

# UNITED STATES PATENT OFFICE.

HARRY S. MORK, OF BOSTON, MASSACHUSETTS, ASSIGNOR TO CHEMICAL PRODUCTS COMPANY, OF BOSTON, MASSACHUSETTS, A CORPORATION OF MAINE.

## ARTICLES COMPOSED OF CELLULOSE ESTERS.

1,074,092.

Specification of Letters Patent.

Patented Sept. 23, 1913.

No Drawing. Original application filed February 10, 1910, Serial No. 543,098. Divided and this application filed May 19, 1910. Serial No. 562,318.

*To all whom it may concern:*

Be it known that I, HARRY S. MORK, a citizen of the United States, residing at Boston, in the county of Suffolk and State 5 of Massachusetts, have invented an Improvement in Articles Composed of Cellulose Esters, of which the following is a specification.

In Letters Patent No. 1,061,771, dated 10 May 13, 1913, a process of treating cellulose esters, such as cellulose acetate, is embodied, consisting essentially in producing a lower cellulose ester of a fatty acid by removing from a higher ester a portion of the 15 combined acid.

In carrying out the process therein set forth the higher ester of the fatty acid is treated with a saponifying agent until a portion of the combined acid is removed.

20 This invention relates to sheets, or films, filaments and the like, composed in part of the lower esters of the fatty acids, as the lower acetates, which also involves the exercise of the invention set forth in my afore- 25 said patent of which this application is a division, yet comprehends new and useful features.

This invention comprises sheets or films and filaments and the like, made of triacetate of cellulose, such as may be prepared 30 according to my Patent #854,374, and such portion thereof as is desired changed by the removal of a part of the combined acid, as hereinafter set forth. Such a sheet or film, 35 filament and the like, is adapted for many uses where the qualities of the triacetate are desirable in some part of the sheet or film, filament and the like, and the qualities of a lower acetate are desirable in other 40 portions thereof. For instance the back of a photographic film base may be composed of the triacetate and the surface composed of a lower acetate; or a pattern on the surface of the base may be composed of a lower 45 acetate; or threads may have an interior of the triacetate and an exterior of a lower acetate; or a part of a film may be changed to the lower acetate from front to back, leaving the remainder unchanged. In short 50 many combinations of this nature may be produced readily involving my invention.

In the process of my application afore- 55 said partial saponification or removal of a

part of the combined acid of the ester is effected in a number of different ways and 55 by the application of usual or suitable saponifying agents, such as sodium or potassium hydroxid, hydrochloric or sulfuric acid, or by some reagents not ordinarily used for the purpose, such as sodium carbonate and ammonia. For example, if cellulose triacetate prepared according to my Patent #854,374, be allowed to stand in aqueous ammonia of specific gravity 0.9 for fifteen or sixteen hours, at a temperature of 60 say 15° to 20° C., saponification will gradually take place, although conversion toward the di-acetate and the monoacetate will not take place in definite stages. These results may likewise be reached by using a stronger 70 solution for a shorter time or the saponification may be carried further if desired by stronger chemicals, greater heat, or longer time or both.

In the present invention the sheets or 75 films, filaments and the like, are treated superficially whereby a portion only of the sheet or film, filament and the like, is changed. Superficial saponification is readily effected by subjecting the portion it is 80 desired to change from the triacetate to a strong hot caustic soda solution or other active saponifying agent for a very short time, as for instance, a 10% sodium hydroxid solution for one or two minutes at 85 60° or 70° C. The saponification will proceed further the longer the reaction is permitted to continue. Or a thin layer of a viscous menstruum, like a starch or gelatin solution containing the active saponifying 90 reagent, may be applied to the surface of the film.

In case it is desired to effect saponification locally in spots or configurations on the surface, the thick solution can be printed upon the film in any desired pattern. For many purposes it is not harmful if the reaction continues so long that the film is superficially saponified until the acid groups have been completely removed. 100

One example where the exercise of my invention is useful is in the treatment of cellulose acetate films for photographic purposes. I have discovered that when such films are partially or superficially saponified 105 they are, by reason of this modification, put

in condition so that the gelatin emulsion or substratum will more readily adhere to them, owing to the increased water absorptive capacity of that portion which has been partially or completely saponified, and the properties of the film may be varied greatly according to the extent of the saponification. Another application is in the case of artificial silk. The number of dyes that can be dyed directly from aqueous solutions on artificial silk made from cellulose triacetate is very limited. When the artificial silk has been subjected to the action of a saponifying agent, in accordance with this invention, I find that by reason of this treatment the number of dyes available for dyeing the material is very materially increased. Another advantage of the exercise of my invention is the fact that even if the original cellulose triacetate is very flexible and strong, the flexibility and strength are noticeably increased by subjecting the triacetate to partial saponification. Furthermore, a sheet or film or a filament superficially saponified by my process is quite distinct from any sheet or film or filament which could be made by attempting to combine two sheets, one made of the triacetate and one of the lower acetate, a thing so impracticable with methods hitherto known, however, that it has not been, to my knowledge, attempted.

The process herein described of preparing sheets, films and filaments for general purposes forms the subject-matter of my application Serial No. 637,857 filed July 11, 1911.

I claim:

1. As a new article of manufacture, a sheet, film or filament composed of an inseparable combination of cellulose of progressively varying degrees of acetylation prepared by removing superficially or locally from the higher cellulose ester a portion of the combined acid.
2. As a new article of manufacture, a sheet, film or filament composed of an inseparable combination of cellulose of progressively varying degrees of acetylation including the triacetate and a lower acetate prepared by removing superficially or locally from the triacetate a portion of the combined acid.
3. As a new article of manufacture, a sheet, film or filament of cellulose triacetate having its surface saponified to produce an

article of progressively varying degrees of acetylation.

4. As a new article of manufacture, a film, filament, sheet or structure composed of cellulose of progressively varying degrees of acetylation and which is physically homogeneous but chemically heterogeneous in its relations to water, dyes and solvents.

5. As a new article of manufacture, a sheet, film or filament composed of cellulose acetate, superficially saponified.

6. As a new article of manufacture, a sheet, film or filament composed mainly of an acetate of cellulose higher than the diacetate and having a surface composed of an acetate of cellulose lower than the triacetate.

7. As a new article of manufacture, a base for a photographic film composed of a cellulose ester, superficially saponified.

8. As a new article of manufacture, a base for a photographic film composed of a cellulose ester, the surface of which is composed of a lower ester than the remainder.

9. As a new article of manufacture, a base for a photographic film composed of a cellulose ester, a portion of the surface of which is composed of a lower ester than the remainder.

10. As a new article of manufacture, a base for a photographic film composed of triacetate of cellulose with a surface composed of a lower acetate of cellulose.

11. As a new article of manufacture, a photographic film-base having a surface of an acetate of cellulose lower than the triacetate and a base of a higher degree of acetylation than the surface.

12. As a new article of manufacture, a base for a photographic film consisting of a support composed of triacetate of cellulose and a surface composed of a lower acetate of cellulose inseparably combined with the support.

13. As a new article of manufacture, a photographic film-base composed of the triacetate of cellulose superficially saponified.

In testimony whereof I have signed my name to this specification in the presence of two subscribing witnesses.

HARRY S. MORK.

Witnesses:

B. J. NOYES,  
H. B. DAVIS.